

Dec. 28, 1948.

H. METTEN ET AL

2,457,781

RAY COUNTER

Filed Jan. 2, 1948

2 Sheets-Sheet 1



Fig. 1

Fig. 3

Fig. 2



Herbert Metten  
Frederic Koury

INVENTORS

BY *Lawrence Brown*,

ATTORNEY

Dec. 28, 1948.

H. METTEN ET AL

2,457,781

RAY COUNTER

Filed Jan. 2, 1948

2 Sheets-Sheet 2



Fig. 4

Herbert Metten  
Frederic Koury

INVENTORS

BY

*Lorraine Brown*

ATTORNEY

## UNITED STATES PATENT OFFICE

2,457,781

## RAY COUNTER

Herbert Metten, Boston, and Frederic Koury, Somerville, Mass., assignors to Sylvania Electric Products Inc., Salem, Mass., a corporation of Massachusetts

Application January 2, 1948, Serial No. 94

8 Claims. (Cl. 250—27.5)

1

This invention relates to ray detection tubes, for example so-called Geiger-Mueller counter tubes, and particularly to such tube for detection of gamma rays.

An object of the invention is a counter tube with increased sensitivity. This object is attained by the use of an annular disc type of counter, in which the discs are plated with bismuth, and particularly with a layer of bismuth in a critical thickness range.

Further objects, advantages and features of the invention will be apparent from the following specification, taken in conjunction with the accompanying drawings, in which:

Figure 1 is a longitudinal section of a device according to the invention;

Figure 2 is a top view thereof;

Figure 3 is a view, partly in section, of one of the annular discs according to the invention; and

Figure 4 is a graph of the coating thickness vs. the sensitivity of the device.

In Figure 1, the metal tube 1 has the end cap 2 fitted to one of its ends, the cylindrical walls 3 of said cap being fitted inside the tube 1 and hermetically sealed thereto. The other end of the tube 1 is sealed by an end cap 4, but at a point removed from the extremity 5 of the tube 1. An exhaust tube 6 is hermetically sealed into end cap 4, and the glass wafer or stem 7 is sealed to said end cap 4 through the intermediary of a "Kovar" metal cylinder and a flanged cylindrical metal piece as shown, the seal being, of course, hermetic.

The lead-in wire 8, sealed through the glass stem 7, ends in the hook 9. Near, but spaced from, the other end of the tube 1 is annular disc 10, at the center of which is the insulating disc 11, of glass or ceramic, for example, flanged to fit the inside of the disc 11, and having a hole 17 at its center through which a wire 12 may be passed with some clearance. The insulating disc 11 has the cylindrical hub 13 around which is fitted a collar 14 with tabs 15 from which the spring wire 16 is bent over the hole 17 and affixed to wire 12, the other end of which is affixed to hook 9. The spring wire 16 holds the central wire 12 reasonably taut. The wire 12 may be of tungsten, for example, and forms the anode of the device.

The lead-in wire 8 and its hooked end 9 are set in a glass tube 20 extending from stem 7 to a position somewhat in advance of the hooked end 9. The annular disc 10 has holes 21 therein, to facilitate exhaust.

2

For example, and not by way of limitation, the tube 1 may be about 2 inches in diameter, with a space of about an inch between end cap 2 and disc 10, and a spacing of about  $\frac{1}{8}$  inch between the annular discs 18, which may have a central opening about half an inch. The wire 12 may be of 0.003 inch diameter. The distance between end caps 2 and 4 may be about 4½ inches. For this particular tube, the drawing is to full scale. The tube has a suitable gas filling.

The annular discs 18 may be of copper, for example, and about 0.008 inch thick, with a bismuth plating about 0.005 to 0.008 inch in thickness. This plating is critical in thickness as shown in Figure 4, the greatest number of net counts per second occurring at about 0.0065 inch thickness of plating. This net count number is nearly 100% greater than that with plain 0.031 inch lead annular discs.

For plating, we have used a solution of 25 grams bismuth trioxide in 125 cc. of 70% perchloric acid, C. P. This is agitated six hours until a colorless solution is formed, and then gradually diluted to one liter with distilled water. As anodes, we used C. P. bismuth metal powder poured into a graphite boat and fired in a hydrogen atmosphere at 800° C. for 15 minutes.

Annular discs of copper or other suitable metal were prepared by degreasing and then soaking in 50% nitric acid solution and then being put in an acid bright dip for 30 seconds. The cleaned discs were then mounted on a clip type plating rack immersed in the plating solution, and plated at a current density of 3 to 9 amperes per square foot for about 16 hours. During plating the parts were agitated with an up and down motion at a rate of about 40 cycles per minute.

After plating the discs were rinsed, treated with 50% nitric acid solution for 30 seconds, then rinsed in water, dried and immediately mounted into the ray detector tube.

The plated surface should be free of stains and bright, with the metallic bismuth deposits of a fine crystal structure, as the density of the plated bismuth is important for the sensitivity of the tube. The density by our plating method is about 0.9 gram per c. c.

The graph of Figure 4 is for a tube as described with a self quenching gas fill, operated at 960 volts in series with a 5 megohm resistor. The tube was tested with an unfiltered radium source 12 inches from the end of the counter. The tube had a starting voltage of about 840 volts with a minimum plateau of 130 volts and a plateau slope of 0.4% per volt rise, over this range.

This tube is several times as sensitive as the conventional concentric cylinder type.

The tube will ordinarily be filled with gas at some convenient pressure, generally about 10 cm. A fill of argon with 0.01% bromine may be used for operating at a lower voltage than that given above. A fill of neon at 20 centimeters of mercury pressure, with the addition, at 0.25 cm. pressure, of a 4 parts argon and 1 part chlorine mixture, is especially good. The tube described in detail herein as an example of a specific embodiment of the invention was filled with about 9½ cm. (of mercury) pressure of argon, and 0.7 cm. pressure of propane, and had 14 discs.

In Figure 3 the copper disc is shown with the plated bismuth layer 22 thereon.

What we claim is:

1. In a ray counter tube having a gas filling and an anode, a cathode comprising a bismuth-plated annular metal disc.
2. In a ray counter tube having a gas filling and an anode, a cathode comprising an annular metal disc having a plating of bismuth between 0.005 and 0.008 inch thick.
3. In a ray counter tube having a gas filling and an anode, a cathode comprising an annular metal disc having a plating of bismuth about 0.0065 inch thick.
4. In a ray counter tube having a gas filling and an anode, a cathode of bismuth substantially 25

5. A gamma ray counter tube comprising a sealed metal envelope, a wire anode along the axis thereof and insulated therefrom, and a series of bismuth-plated annular discs coaxial with said wire and in contact with said envelope.

6. In a gamma ray counter tube having a gas filling and an anode, an annular copper disc plated with bismuth to a thickness of about 0.0065 inch.

10 7. A gamma ray counter tube comprising a sealed metal envelope, a wire anode along the axis thereof and insulated therefrom, a series of bismuth-plated annular discs coaxial with said wire and in contact with said envelope, and a gas filling at a pressure of about 10 cm. of mercury therein, said gas filling comprising argon with about 0.01% bromine.

15 8. In a ray counter tube having a gas filling and an anode, a metal cathode having a plating of bismuth about 0.0065 inch thick.

HERBERT METTEN.  
FREDERIC KOURY.

#### REFERENCES CITED

The following references are of record in the file of this patent:

#### UNITED STATES PATENTS

30 Number Name Date  
2,397,071 Hare ----- Mar. 19, 1946